

Patented Dec. 14, 1926.

1,610,362

# UNITED STATES PATENT OFFICE

THOMAS WATTS COSLETT, OF BIRMINGHAM, ENGLAND.

## PROCESS FOR THE TREATMENT OF IRON OR STEEL FOR PREVENTING OXIDATION OR RUSTING.

No Drawing. Application filed February 6, 1926, Serial No. 86,662, and in Great Britain June 26, 1925.

This invention relates to the treatment of iron or steel or articles composed or having a surface of iron or steel by processes of the kind described in my prior United States patent specifications Nos. 870,937 and 1,007,069 according to which the iron or steel surfaces are provided with a protective covering or deposit of a compound that renders the said surfaces capable of resisting or being unaffected by the action of moisture or other oxidizing or "rusting" influences. In the processes in question the iron or steel or the articles composed or having a surface of iron or steel is or are subjected to the action of a dilute solution of phosphoric acid either alone or with the addition of a suitable substance such as iron filings, ferrous phosphate, or other appropriate compound adapted to control or regulate the chemical action upon the metal or articles undergoing treatment, or of phosphoric acid in the presence of zinc or a suitable zinc compound, or of a solution thereof in phosphoric acid, or of a solution of acid zinc phosphate (that is zinc phosphate solution with a small excess of phosphoric acid), or of a solution containing zinc phosphate and iron phosphate.

According to the present invention a process of the kind referred to for the treatment of iron or steel or articles with an iron or steel surface consists in subjecting it or them to the action of a solution of one or other of the kinds hereinbefore referred to and containing as an additional constituent a compound of boron, for instance boric acid or a borate such for example as borax, care being exercised to select a boron compound such as will not detrimentally affect the deposit on the iron or steel. Preferably the solutions employed for the present process should be only slightly acid; as an illustration it may be mentioned that a suitable acidity of a bath of zinc phosphate solution, before the addition of the boric acid thereto, is such that 10 cubic centimetres of the solution require about 4.8 to 5.5 cubic centimetres of deci-normal sodium hydroxide solution for their neutralization.

For the treatment of articles by the improved process according to the present invention there may be taken as an example of a suitable bath solution one prepared by dissolving pasty or concentrated acid zinc phosphate and boric acid (powdered or crys-

tals) in water, in the approximate relative proportions of about 2 ounces of the phosphate and 1½ ounces boric acid to one gallon of water.

For the preparation of the pasty or concentrated acid zinc phosphate a suitable method is to dissolve 6 ounces finely granulated or powdered zinc in ½ pint phosphoric acid B. P. and ½ pint hot water—the solution is set aside for a few hours, 65 stirred, and a pasty or powdered mass suitable for use in making up the bath solution in the proportions previously mentioned is obtained.

The treatment of the iron or steel or articles with an iron or steel surface is preferably carried out with a hot solution and in order to diminish loss of boric acid therefrom due to its volatility in steam, the vessel in which it is contained and wherein the 70 treatment of the iron or steel articles is carried out should be kept covered as much as possible so as to reduce evaporation to a minimum. To prevent undue diminution in the concentration of boric acid present in 75 the bath solution during the treatment operation, an additional amount of boric acid may be added from time to time so as to compensate for that lost by evaporation and keep the amount of boric acid in the solution 80 as constant as possible. Other ingredients of the solution when required may also be added to the bath from time to time to replace those used up in carrying out the process.

A suitable method for determining the approximate quantities of acid zinc phosphate and boric acid contained in the bath solution is as follows: 10 cubic centimetres of the bath solution are titrated with a deci-normal solution of sodium hydroxide using phenolphthalein as an indicator. The fresh bath prepared with the quantities of acid zinc phosphate and boric acid mentioned above requires about 6.5 to 7 cubic centimetres of the sodium hydroxide solution, the increase of about 1 to 1.5 cubic centimetres over the titration figure obtained in the case of a bath of zinc phosphate solution alone being due to the presence of the boric acid. 95 After reading the burette there is added to the vessel containing the rose coloured solution about 30 cubic centimetres of a neutralized calcium chloride solution prepared by dissolving about 100 grammes of calcium 100 chloride in 110

chloride in 150 cubic centimetres of water, whereupon the rose colour will be discharged. The sodium hydroxide solution is then again run in from the burette until the rose colour reappears and remains permanent after a thorough shaking. In the case of the fresh bath solution about a further 13 cubic centimetres of the deci-normal sodium hydroxide solution will be required, thus making a total of 20 cubic centimetres for the two titrations. The first titration figure obtained, after making an allowance of about 1 to 1.5 cubic centimetres for the boric acid present, measures approximately the amount of acid zinc phosphate present, and the second figure obtained (13 cubic centimetres for the fresh bath) measures approximately the amount of boric acid present. By titrating a sample portion of the bath in this manner the quantities of acid zinc phosphate and boric acid present at any time can be approximately ascertained and from the results obtained the desired quantities of ingredients can be added to the bath solution when necessary to renew its strength.

Before treating the articles in the solution they may previously be immersed for a short period, say a few minutes, in a hot or cold solution of boric acid of about five per cent or less concentration.

The articles to be treated may be suspended in the solution on iron or zinc wires or on holders or in containers made of any suitable material that has no detrimental effect on the solution.

The formation of the deposit on the iron or steel or surface under treatment may be assisted if desired by passing an electric current through the solution; when this procedure is adapted a cathode of zinc, iron or steel should be employed and the article to be treated should be made the anode.

By the use of a solution containing boric acid or a borate in accordance with the present invention the uniformity and adherence of the deposit obtained on the iron or steel are much enhanced, and the treatment is rendered very much more rapid as deposits can be obtained in a few minutes which are even more effective for rendering the surface of the article treated non-oxidizable or rust-proof than the deposits for which a period of about 1½ hours' treatment was required with the solutions heretofore employed. Further considerable saving results from the process owing to deposits of the desired character being obtained in much less time and with much less depletion of the constituents of the solution than was hitherto possible.

What I claim and desire to secure by Letters Patent of the United States is:—

1. A process of the kind referred to for the treatment of iron or steel or articles

composed or having a surface of iron or steel which consists in subjecting the same to the action of an aqueous solution of acid zinc phosphate and boric acid in the relative proportions of about two ounces of the phosphate and one and one third ounces of the boric acid to one gallon of water, for the purpose specified.

2. A process for the treatment of iron or steel or articles composed or having a surface of iron or steel for preventing the oxidation or rusting thereof which consists in subjecting the same to the action of a solution of phosphoric acid and a compound of boron.

3. A process for the treatment of iron or steel or articles composed or having a surface of iron or steel for preventing the oxidation or rusting thereof which consists in subjecting the same to the action of a zinc-containing and boron-containing solution of phosphoric acid.

4. A process for the treatment of iron or steel or articles composed or having a surface of iron or steel for preventing the oxidation or rusting thereof, which consists in subjecting the same to the action of a dilute zinc-containing and boron-containing solution of phosphoric acid.

5. A process for the treatment of iron or steel or articles composed or having a surface of iron or steel for preventing the oxidation or rusting thereof which consists in subjecting the same to the action of a zinc-containing and boron-containing solution of phosphoric acid of varying degrees of concentration.

6. A process for the treatment of iron or steel or articles composed or having a surface of iron or steel for preventing the oxidation or rusting thereof which consists in subjecting the same to the action of a solution of phosphoric acid and a compound of boron with the addition of a substance adapted to control or regulate the chemical reactions.

7. A process for the treatment of iron or steel or articles composed or having a surface of iron or steel for preventing the oxidation or rusting thereof, which consists in subjecting the same to the action of a dilute solution of phosphoric acid and a compound of boron with the addition of a substance adapted to control or regulate the chemical reactions.

8. A process for the treatment of iron or steel or articles composed or having a surface of iron or steel for preventing the oxidation or rusting thereof which consists in subjecting the same to the action of a solution containing zinc and iron phosphate and a compound of boron.

9. A process for the treatment of iron or steel or articles composed or having a surface of iron or steel for preventing the oxidation or rusting thereof, which consists in subject-

- ing the same to the action of a dilute solution containing zinc and iron phosphate and a compound of boron.
10. A process for the treatment of iron or steel or articles composed or having a surface of iron or steel for preventing the oxidation or rusting thereof which consists in subjecting the same to the action of a dilute solution of phosphoric acid and a compound of boron.
11. A process for the treatment of iron or steel or articles composed or having a surface of iron or steel for preventing the oxidation or rusting thereof which consists in subjecting the same to the action of a zinc-containing and boric-acid-containing solution of phosphoric acid.
20. A process for the treatment of iron or steel or articles composed or having a surface of iron or steel for preventing the oxidation or rusting thereof which consists in subjecting the same to the action of a solution of phosphoric acid and boric acid with the addition of a substance adapted to control or regulate the chemical reactions.
30. A process for the treatment of iron or steel or articles composed or having a surface of iron or steel for preventing the oxidation or rusting thereof, which consists in subjecting the same to the action of a dilute solution of phosphoric acid and boric acid with the addition of a substance adapted to control or regulate the chemical reactions.
35. A process for the treatment of iron or steel or articles composed or having a surface of iron or steel for preventing the oxidation or rusting thereof which consists in subjecting the same to the action of a solution containing zinc and iron phosphate and boric acid.
45. A process for the treatment of iron or steel or articles composed or having a surface of iron or steel for preventing the oxidation or rusting thereof which consists in subjecting the same to the action of a dilute solution containing zinc and iron phosphate and boric acid.
50. A process for the treatment of iron or steel or articles composed or having a surface of iron or steel for preventing the oxidation or rusting thereof which consists in subjecting the same to the action of a dilute solution of phosphoric acid and boric acid.
55. A process for the treatment of iron or steel or articles composed or having a surface of iron or steel for preventing the oxidation or rusting thereof which consists in subjecting the same to the action of a solution containing acid zinc phosphate and boric acid in or about the proportions hereinbefore stated.
60. A process as in claim 1, in which before subjecting the articles to the treatment with the solution they are immersed for a short period in a solution of boric acid.
19. A process as in claim 2, in which before subjecting the articles to the treatment with the solution they are immersed for a short period in a solution of boric acid.
20. A process as in claim 3, in which before subjecting the articles to the treatment with the solution they are immersed for a short period in a solution of boric acid.
70. 21. A process as in claim 6, in which before subjecting the articles to the treatment with the solution they are immersed for a short period in a solution of boric acid.
75. 22. A process as in claim 8, in which before subjecting the articles to the treatment with the solution they are immersed for a short period in a solution of boric acid.
80. 23. A process as in claim 10, in which before subjecting the articles to the treatment with the solution they are immersed for a short period in a solution of boric acid.
85. 24. A process as in claim 13, in which before subjecting the articles to the treatment with the solution they are immersed for a short period in a solution of boric acid.
90. 25. A process as in claim 14, in which before subjecting the articles to the treatment with the solution they are immersed for a short period in a solution of boric acid.
95. 26. A process as in claim 1, in which an electric current is passed through the solution during the treatment therewith of the iron or steel or articles with an iron or steel surface for the purpose specified.
100. 27. A process as in claim 2, in which an electric current is passed through the solution during the treatment therewith of the iron or steel or articles with an iron or steel surface for the purpose specified.
105. 28. A process as in claim 10, in which an electric current is passed through the solution during the treatment therewith of the iron or steel or articles with an iron or steel surface for the purpose specified.
110. 29. A process as in claim 14, in which an electric current is passed through the solution during the treatment therewith of the iron or steel or articles with an iron or steel surface for the purpose specified.
115. 30. In the treatment of iron or steel or articles composed of iron or steel a compound consisting of a dilute solution of phosphoric acid and a compound of boron.
120. 31. In the treatment of iron or steel or articles composed of iron or steel a compound consisting of a zinc-containing and boron-containing solution of phosphoric acid.
125. 32. In the treatment of iron or steel or articles composed of iron or steel a compound consisting of a solution containing zinc and iron phosphate and a compound of boron.
33. In the treatment of iron or steel or articles composed of iron or steel a compound consisting of a solution containing acid zinc phosphate and boric acid.

THOMAS WATTS COSLETT.